

# United States Patent Office

3,349,522

Patented Oct. 31, 1967

1

3,349,522

SPINNERET SURFACE FINISHING  
James Stanley Cobb, Jr., Martinsville, Va., assignor to  
E. I. du Pont de Nemours and Company, Wilmington,  
Del., a corporation of Delaware  
No Drawing. Filed July 27, 1965, Ser. No. 475,238  
3 Claims. (Cl. 51—324)

## ABSTRACT OF THE DISCLOSURE

After normal fabrication steps which leave protuberances, the face of a spinneret is finished by abrading it to remove the protuberances, polishing the abraded face on a "long nap" cloth to remove burrs, lapping the face and then polishing it on a "no nap" cloth.

This invention relates generally to the extrusion of viscous organic materials and more particularly to procedures involved in the fabrication of spinnerets adapted for use in the spinning of synthetic filaments.

Experience has shown that a sharp edge is needed at the exit of each spinneret capillary to insure a better and more uniform product. Sharp edges also improve wiping efficiency. Wiping is the removal during a spinning interruption of the organic stalactites which form at the capillary exits during the spinning process. It further has been found that a bright finish on the spinneret face is desirable for prevention of corrosion at these sharp edges.

Normally, the method used to form capillaries in a spinneret blank is to either drill or punch or use a combination of these steps, leaving protuberances or burrs on the face of the spinneret. These protuberances are removed by abrading the spinneret face, e.g., by lapping, grinding, or rubbing on abrasive paper. All of these steps put a burr on the inside edge of each capillary. When such burrs are removed with a sizing punch or broach, another lapping, grinding, or rubbing step is required to remove the metal forced out to the face of the spinneret by the broaching step. Instead of removing burrs with a sizing punch or broach, burr formation within the capillary is sometimes avoided by plugging each capillary with glass or metal inserts before removal of the protuberances. The inserts are not removed until completion of the surface-finishing steps. Both of these techniques are time consuming and costly.

The major objective of this invention is to provide an improved finishing technique for removal of burrs from capillary walls while providing a bright finish on the face of a spinneret and sharp edges at the capillary exits. Another objective is to provide a less-costly technique for finishing spinnerets. More specifically, the object of this invention is to avoid the use of sizing punches, broaches or capillary plugs in the fabrication of capillaries which are not only free from internal burrs but also have sharp exits.

With these and other objects in view, the presently disclosed method comprises generally the steps of machining capillaries which exit at the face of a spinneret blank, removing protuberances left on the face of the blank during the machining step by abrading, removing the burrs formed inside the capillaries during the protuberance removal step by polishing on a "long nap" cloth, resharpening the exits of the capillaries by lapping, and putting a bright finish on the spinneret face by polishing on a "no nap" cloth.

Any of the known techniques can be used to form a spinneret plate or blank and to form the lead-in holes and capillaries, e.g., the spinneret punching machine described by Thomann et al. in U.S. 2,709,492. After all of the capillaries are punched, there are a number of protuber-

2

ances remaining on the face of the spinneret. Depending upon the technique used, either the capillary is partially opened in this protuberance or, using the technique described by Thomann et al., the capillary does not break through the protuberance.

After the punching is completed for all the capillaries, the finishing technique of this invention calls for removal of the protuberances by an abrading step, e.g., by lapping, grinding, or rubbing (by hand or mechanically) on a fine abrasive sheet. The abrasive sheet is mounted on a flat plate so that, in addition to removing the protuberances, the face of the spinneret is made flat. However, this step leaves a scratched surface and, in addition, removal of the protuberance usually leaves a burr inside the capillary. The next step is to place the spinneret face down on a metal wheel covered by a "long nap" felt cloth. The polishing wheel is then rotated and the spinneret reciprocated on the wheel so that a uniform multi-directional cut is achieved. It is also sometimes desirable to rotate the spinneret as well as the polishing wheel. While the mechanism is not completely understood, it is believed that the fibers or filaments of the "long nap" reach up into the capillary and pull or abrade away the burrs inside the capillary. This step is continued until the burrs are removed. However, in doing this, the edge or exit of the capillary to the face of the spinneret becomes rounded. It is now necessary to lap the face of the spinneret to be sure that it is flat and to sharpen the capillary exits. However, this does not put on the high or bright finish that is necessary to achieve good corrosion resistance. Consequently, a final polishing step is carried out with a rotating "no nap" cloth.

A typical example is the fabrication of a spinneret for spinning nylon filaments from type 430 stainless steel, which spinneret has round capillaries 0.009 inch in diameter and 0.012 inch long. Drilling a lead-in hole in the spinneret blank is the first step in the preparation of each capillary. In a series of drilling and punching steps, the final capillary is formed but does not break through a protuberance left on the spinneret face. This protuberance or burr is removed manually by rubbing the spinneret on 400 grit and then on 600 grit wet paper (mounted on a flat plate) until all the burr is gone. This step, however, leaves a rough capillary exit, that is, there are scratches on the face of the spinneret which run through the capillary and burrs are bent into the capillary. The burrs are removed by polishing on a rotating metal wheel, i.e., a metal wheel which is covered with a "long nap," plucked pile cloth of uniform, sheared, 100% virgin wool ("Knoxall" No. 1,118 napped cloth, manufactured by E.H. Beste Company, Boston, Mass.). After the cloth has been charged with chrome rouge and a light machine oil, this step is continued until the burr is removed, normally approximately five minutes. Burr removal leaves the hole edge rounded to an 0.000080" to 0.000150" radius. This radius is measured by an interference microscope. The next step is a micro-lapping operation in which the spinneret is placed in a lapping machine (the Lapmaster made by John Crane Company) which has a wheel on which the spinneret plate is placed and constrained by a ring-shaped holder. With a weight on the plate, it walks around the inside periphery of the holder as the wheel is rotated. In the preferred method, this is accomplished by using a 0.5 to 1.0 p.s.i. lapping pressure with a five micron (grit size) compound in a mixture of light oils similar to kerosene (No. 3 Lapping Vehicle, John Crane Company) and the lapping continued for approximately seven minutes. The time required to lap the hole edge sharp is a function of the lapping pressure and the number of interference rings. In general, the lapping pressure is adjusted so that the lapping time is

approximately thirty seconds per interference ring. An alternative to this is to use a coarser compound, e.g., 1,700 grit compound, for approximately one minute. Care must be taken to insure that this micro-lapping is not done too long, otherwise this step will put a burr back into the capillary. The final polishing step is accomplished by using a "no nap" cloth on the polishing wheel. A nylon satin, charged with chrome rouge and a light machine oil, is used in this example. The result is a burr-free edge with a radius between 0.000010" and 0.000050".

Depending upon the materials of construction, it is of course obvious that various times and abrasives could be used. It should also be apparent that the techniques disclosed herein can be used for capillaries with odd-shaped cross sections. Other adaptations and modifications inherent in the practice of this invention will occur readily to those skilled in the art and, accordingly, its extent is intended to be limited only by the scope of the appended claims.

Having thus described the invention, what is claimed as new and desired to be secured by Letters Patent is:

1. In a spinneret fabrication method including the preliminary step of machining a capillary hole in a spinneret blank thereby leaving a protuberance on one face of the spinneret blank, a finishing technique comprising the steps of: abrading said face to remove the protuberance; polishing the abraded face on a long nap cloth to remove burrs from within said hole; lapping said face just sufficiently to sharpen the hole exit; and polishing the face on a no nap cloth.

2. In a spinneret fabrication method including the

preliminary step of machining at least one capillary hole in a metal spinneret blank thereby leaving a protuberance on one face of the spinneret blank, a finishing technique comprising the steps of: rubbing said face on an abrasive sheet to remove said protuberance; polishing the abraded face on a rotating wheel covered with a long nap felt cloth; lapping the polished face just sufficiently to sharpen the hole exit; and polishing said face on a no nap cloth.

3. In a spinneret fabrication method including the preliminary steps of machining a plurality of capillary holes in a spinneret plate thereby leaving protuberances on one face of the spinneret plate, a finishing technique comprising the steps of: rubbing said face on a flat plate covered with an abrasive sheet; polishing said face on a rotating metal wheel covered with a long nap cloth previously charged with chrome rouge and a light machine oil, thereby removing burrs from within the capillary holes but leaving rounded edges at the capillary hole exits; lapping the polished face just sufficiently to sharpen said edges; and polishing said face on a rotating wheel covered with a no nap cloth.

#### References Cited

##### UNITED STATES PATENTS

|    |           |         |                |       |          |
|----|-----------|---------|----------------|-------|----------|
| 25 | 1,952,025 | 3/1934  | White          | ----- | 18-8     |
|    | 2,115,402 | 4/1938  | Spaanbroek     | ----- | 51-323 X |
|    | 2,658,414 | 11/1953 | Issartial      | ----- | 51-323 X |
|    | 2,709,492 | 5/1955  | Thomann et al. | ----- | 72-1     |
| 30 | 2,923,969 | 2/1960  | Thorpe         | ----- | 18-8     |

LESTER M. SWINGLE, *Primary Examiner.*